

Oct. 9, 1956

H. L. CROWLEY ET AL  
PROCESS OF FORMING POWDERED METAL PARTS IN ATMOSPHERE  
CONTAINING HBr AND ARTICLES RESULTING THEREFROM  
Filed March 7, 1952

2,765,519

Fig. 1



Fig. 2



LEGEND  
 $\left\{ \begin{array}{l} + = 0.0 \\ \times = 0.5 \\ \circ = 1.0 \\ \bullet = 5.0 \\ * = 10.0 \\ \circ = 15.0 \end{array} \right\} \% \text{ HBr}$

INVENTORS  
Henry L. Crowley  
BY Marion Ernest Graham

Robert S. Dunham

ATTORNEY

**PROCESS OF FORMING POWDERED METAL PARTS IN ATMOSPHERE CONTAINING HBr AND ARTICLES RESULTING THEREFROM**

Henry L. Crowley, South Orange, N. J., and Marion Ernest Graham, Parma, Ohio, assignors, by direct and mesne assignments, to Republic Steel Corporation, Cleveland, Ohio, a corporation of New Jersey

Application March 7, 1952, Serial No. 275,382

17 Claims. (Cl. 29—182.5)

The present invention relates to a process of heat treating powdered metal parts and more particularly to heat treating and/or sintering such parts formed by pressing powdered metal into a desired shape in order that the parts, as heat treated or sintered, shall have the desired physical characteristics. The present invention also relates to parts such as those which are formed by the present process.

The present application is related by similarity of subject matter to our prior and copending application, Serial No. 166,312, filed June 6, 1950, now abandoned and entitled Process of Heat Treating Powdered Metal Parts and Parts Formed Thereby. Said application Serial No. 166,312 was followed by a continuation-in-part thereof, Serial No. 300,908, filed July 25, 1952, which had the same title as Serial No. 166,312. This application is now abandoned but has been replaced by a further application Serial No. 575,794, which was copending with Serial No. 300,908 and is a continuation-in-part thereof. Serial No. 575,794 has the title Process of Heat Treating Powdered Metal Parts. The line of demarcation between these two inventions is based on the principle that when the atmosphere in which the parts are sintered contains HCl, the subject matter is included in said application, Ser. No. 575,794; while the present case is restricted to those situations wherein the sintering atmosphere contains HBr.

In the past, it has been customary in the making of parts by so-called "powder metallurgy" practices to select the powder of one or more metals, mix if powders of more than one metal are used, compact this powder in a suitable mold under relatively high pressure, then sinter the pressed parts in a non-oxidizing atmosphere at a suitable temperature, which is chosen in respect to the composition of the parts, in order that the metal powder shall be bound together into the desired article. Parts so formed are usually not as strong as a part made from cast metal of substantially the same chemical composition respectively, but they have the advantage that little or no machining need be done following the formation of the desired part in this way. As a result, the parts may be given adequate mechanical strength for some particular purposes, not requiring the strength of cast metal parts, and at the same time be made much quicker and cheaper. Such prior art processes have been applied using single metals and using combinations of metals, usually by mixing the powders of two or more metals in desired proportions. The atmospheres in which the heat treating or sintering has been done are uniformly non-oxidizing in character, but within that limitation, have been of many different types. All this prior art practice is now quite well known and is described in numerous text books on the subject.

The present invention improves this prior art practice in a substantial manner in that parts may be formed and heat treated in accordance with the present invention, so as to have greatly enhanced physical properties, for example, tensile strength and elongation, when heat treated

at the same temperatures that would have been used in accordance with prior art practices. Alternatively, at least as good physical properties may be imparted to a given part as in the prior art, while using substantially lower temperatures for the heat treating than was thought possible in accordance with prior art practices. Intermediate results may be obtained in accordance with the present invention, including somewhat enhanced physical properties as aforesaid, while using somewhat lower temperatures than were considered standard in accordance with the prior art teachings.

Summarizing the present invention, the processes in accordance therewith all involve heat treating in an atmosphere containing at least about 1% HBr by volume. 15 Although it has been found that the addition of amounts of HBr, less than about 1% by volume to the sintering atmosphere, are of little, if any, advantage and in some cases are even deleterious to the physical properties of the part sintered therein; at concentrations of at least about 1% HBr and above in the atmosphere, the improvements in physical properties of the parts made according to the present process are more or less proportionate to the concentration of HBr in the atmosphere about the parts during the heat treatment up to about 5% HBr concentration in this atmosphere by volume. 20 The enhanced characteristics of the final product have been found to reach their peaks at about 5% to about 15% by volume of gaseous HBr in the atmosphere, so that it is pointless to use any higher percentage and, in fact, from some points of view, as hereinafter set forth, the use of higher concentrations of HBr may be undesirable.

Metals which are susceptible of being formed into parts, in accordance with the present invention, are broadly, relatively difficultly bromidizable metals, namely, one or more metals selected from the group consisting of iron, nickel, cobalt, copper, lead, cadmium, tin and molybdenum. On the other hand, relatively easily bromidizable metals, such as zinc, aluminum and magnesium are not susceptible to use as the metals or as one of the metals present to any substantial extent at least, of parts which may be heat treated in accordance with the present invention. Further details of the present invention will be brought out more specifically hereinafter and will be illustrated by actual examples of the present process.

The present invention also includes the products made in accordance with the present process, which are characterized by substantially greater tensile strength than 50 similar articles made by the identical process, with the exception that the sintering atmosphere contains less than about 1% by volume of HBr or is substantially free of HBr. Such novel products of the present process are usually also characterized by substantially greater elongations under tension in respect to similar articles.

Considering now details of the present invention and the principles governing it, there will be discussed first the metal or metals which may be used in accordance with this invention. Broadly, as aforesaid, the metals usable 60 are practically restricted to those metals which are relatively difficult to bromidize. The list of such appropriate metals is given above. This list includes all the metals now known to be usable, singly or in combination, in metal parts which may be processed in accordance with the present invention. In the event that some one of the relatively easily bromidizable metals, such as zinc, aluminum or magnesium, be present in any substantial amount, either alone, as an ingredient of a mixture, or as one metal forming an alloy with some other metal or metals 65 which may be in the acceptable list given above, trouble is encountered. For example, brass, an alloy consisting of copper and zinc, is not susceptible of use when such

alloy powder is used in forming the parts to be made, for the reason that the zinc tends to bromidize easily and defeats the purpose to be attained by the present invention as aforesaid. In contrast to this, bronze powders, consisting of copper and tin, both in the acceptable group, may be formed and heat treated in accordance with the present invention as will appear more particularly from the examples hereinafter given.

The present invention is applicable when one or more metals are used, whether the metals, if two or more, be introduced as separate powders of the individual metals or as alloy powders, i. e., wherein each particle of the powder is an alloy. When separate powders of individual metals are originally used in making the parts, there is considerable evidence that there is increased inter-diffusion of the metal particles when operating in accordance with the process of the present invention as compared with prior art processes.

The theory, which is now believed to be basically correct, but is not particularly relied upon in support of the patentability of the appended claims, is that when relatively large amounts of HBr are present in the atmosphere during heat treating, relatively easily bromidizable metals are attacked by the HBr to such an extent that the final product has present therein substantial amounts of the bromides of the easily bromidizable metals and/or is porous due to the volatilization of such bromides, leaving spaces formerly occupied by the bromidized metals. In either event, there results a product, different in composition from the metal powder which was subjected to the pressing operation and introduced into the heat treating step, which product has, in fact, less desirable physical characteristics than would be present if prior art practices were employed, using a non-oxidizing atmosphere without HBr present therein. The process may, therefore, be said to be applicable to the metals—iron, nickel, cobalt, copper, lead, cadmium, tin and molybdenum or to mixtures or alloys thereof, as far as is now known.

The next major factor to be considered in the present case is the atmosphere which is to be used during the heat treating. This atmosphere must be essentially non-oxidizing in character. It may be neutral or reducing, but cannot be, to any substantial extent, oxidizing. Many such atmospheres (absent HBr) have been tried in the prior art, so that no particular details need be given here of the large number of different possible non-oxidizing atmospheres which are usable. It is found that nitrogen, a neutral gas, is operative as the non-oxidizing atmosphere. It has been found, however, that when the atmosphere surrounding the parts during the heat treatment used is reducing in character, such as gas containing a substantial amount of or consisting entirely of hydrogen (other than the HBr present therein), better results are obtained than with a strictly neutral gas. Thus, the preferred atmosphere, in accordance with the present invention, is one in which there is a substantial proportion of hydrogen. The theories now available tending to explain this will be set forth hereinafter.

The essential distinction between the present invention and the prior art is in the use of some gaseous HBr (at least about 1% by volume) as a part of the atmosphere surrounding the metallic parts during the heat treatment thereof. It is found that when this process is carried on, the parts as finally made and as a result of the heat treatment, have enhanced physical characteristics of tensile strength and elongation, in respect to articles made in the same way throughout, with the exception that the atmosphere in which they are heat treated contained no HBr or amounts thereof of less than about 1% by volume. These differences will be apparent from particular examples hereinafter given and from the accompanying drawings.

The advantages to be gained by the presence of HBr in the gas surrounding the articles in the heat treatment is more or less proportionate to the concentration of

HBr, provided that at least about 1% HBr by volume is present. Concentrations of HBr substantially less than about 1% have been found adversely to affect the physical characteristics of the articles. However, as long as at least about 1% HBr by volume is present, greater advantages are gained by using higher percentages of HBr until concentrations of about 5% to about 15% (by volume) are reached. In this range of concentrations, a plot of the value of certain physical characteristics against

10 HBr concentration levels off. Based upon plots of this kind, such as are shown in the accompanying drawings, it is the principle of this invention that any amount of HBr above about 1% by volume is advantageous. Preferred ranges, however, of concentration of HBr, in accordance with the present invention are from about 1% to about 15% by volume. For maximum advantages from the point of view of physical characteristics of the final product, in accordance with the present invention, the range of about 5% to about 15% is found to be preferred. Beyond 15% there seems to be no purpose in increasing HBr concentration, as the cost of the operation is increased to some extent and the physical properties of the final product, not substantially better. In addition to this, as the concentration of HBr in the gas 20 is raised, the tendency toward bromidizing some of the metal present is correspondingly increased.

This point is related to the theories now believed to be correct for the use of atmospheres containing some reducing gas as hydrogen. Taking iron, for example, there is 25 a progressively increasing tendency, as the HBr concentration is increased, for a reaction to occur between iron and the HBr to form ferrous bromide. If any ferrous bromide be formed, even instantaneously, any hydrogen present in the gas will tend to reduce it to reform iron and 30 to liberate HBr in gaseous form. Thus, from an overall point of view, the presence of hydrogen in the atmosphere tends to prevent the formation and possible subsequent volatilization of ferrous bromide. Corresponding reactions can occur between other metals present and 35 HBr. For this reason, it is usually preferred to keep as low an HBr concentration as possible consistent with obtaining desired results, provided, of course, that the concentration of HBr be kept at at least 1% by volume, while 40 at the same time having present in the gas some hydrogen. Another factor to be considered is the tendency for gas 45 containing HBr to corrode apparatus in which the process is carried on. Here again, in order to minimize such corrosion, it is usually desirable to use as low a concentration of HBr as can be used (provided it is at least 1% by volume), while still obtaining the advantages of the 50 present invention in producing articles having enhanced physical properties.

In contrast with the above, it is the present theory that 55 when HBr is used in accordance with the present invention in an atmosphere consisting, apart from HBr, of a neutral gas such as nitrogen, there are opposing effects. The presence of HBr will give enhanced physical characteristics in the final product, in accordance with the present invention. On the other hand, the presence of HBr in the absence of a strongly reducing gas, such as hydrogen, will result in some bromidizing of the metal. This, in turn, will result in relatively less desirable physical properties. The net result is believed to be a balance between these two effects.

Several theories have been expressed tending to explain 60 the novel and highly beneficial results obtained from the practice of the present invention. One of these theories is that the HBr present acts in a manner similar to a pickling bath in that it serves to clean the surface of the metallic particles by removing any oxide film therefrom. This leaves the particles with clean surfaces, which are 65 enabled more efficiently to sinter together, so as to form a superior article under a given set of conditions. The removal of the oxides thus results in enhanced physical 70 characteristics in the final article.

Another theory, which has been expressed and which perhaps partakes of the first expressed theory to some extent, is that the HBr present in the gas reacts with any metal oxides present to convert them to the respective bromides. These bromides, in a process employing a gas containing some hydrogen, may be reduced; and the reduced metal so formed may then act as a cement or binder to bind the particles of the original material together. In such an event, the HBr acts in effect as a catalyst, as it is regenerated by the reduction reaction with hydrogen.

Although the process of the present invention, namely, sintering in an atmosphere containing at least 1% HBr by volume, has been found to be similar in some respects to our copending application, Serial No. 166,312 aforesaid, it is to be noted that while in our former application it was found that the enhancement of certain physical properties, such as tensile strength, has been found more or less proportional to HCl present in the sintering atmosphere up to about 15%, this is not the case when the sintering is carried out in an atmosphere containing HBr according to the present invention. It has further been found and will be particularly illustrated by specific examples, that the presence of small amounts of HBr in the sintering atmosphere, namely, amounts substantially less than about 1% by volume, not only fail to enhance the physical properties of the parts being treated, but actually have a substantial adverse effect on those properties. At concentrations of about 1% or more by volume of HBr and up to about 5%, it is found that the enhancement of physical properties is substantially proportional to the concentration of HBr. No explanation is known at the present time for the apparently anomalous behaviour of HBr when present in concentrations of substantially below 1% by volume. Thus, in the present invention, the lower limit of HBr concentration is somewhat critical as will be illustrated by subsequent examples.

While the theories herein are now believed to be correct, the patentability of the appended claims is not predicated upon the correctness of these theories; but rather upon the novel combination of process steps and the novel product specifically recited herein. It is not known exactly why these improved results occur. It is known, however, that they do in fact occur and that they are reproducible when the teachings of this application are followed. It appears that the HBr must be present in gaseous form in the atmosphere surrounding the articles. This was proven by the fact that while gaseous HBr was effective in securing enhanced physical properties in an iron body or article, no desirable results were attained when using a reducing atmosphere as in the prior art and when bromide was supplied in the form of solid ferrous bromide intermixed with iron powder as a part of the article to be heat treated. This was so even when the atmosphere used surrounding the ferrous bromide containing article consisted solely of hydrogen. This result was surprising in view of the fact that it is known that in an atmosphere of hydrogen, ferrous bromide may be reduced to metallic iron at the temperature at which this article was held for heat treatment. Under the circumstances of the test, wherein the powdered iron article contained solid  $FeBr_2$ , the article produced had a lower strength as compared with an article formed of powdered iron and heat treated in accordance with the prior art at the same temperature. From this, it was concluded that in order to attain the desired results of the present process, it is not feasible to supply a bromide, as solid ferrous bromide, admixed in the article itself, so that HBr must be otherwise supplied to, or be present in, the gases surrounding the article during heat treatment.

It has further been found that while a bromide, such as  $FeBr_2$ , intermixed with the metallic material being sintered, exerts an undesired influence upon the tensile strength of the resulting sintered article, the presence of gaseous HBr in the sintering atmosphere always exerts a beneficial influence, even when some bromide is present in an intermixed condition. Intermixed bromide can-

not properly be relied upon to provide HBr in the gases even when a reducing gas, such as hydrogen, is present; but such HBr must be provided from a separate source. Thus the amount of bromides intermixed in the metallic material should be minimized in order to minimize the deleterious effect thereof on the tensile strength of the articles being made. At the same time the undesired effects of the presence of small amounts of bromide in the metallic material being sintered (such as might be present as an impurity) may be compensated for by providing an ample amount of HBr in the sintering atmosphere which is supplied from a source independent of intermixed bromide or bromine-containing material.

The next and last major factor to be considered in the present process is the temperature at which the heat treating takes place. In accordance with the prior art wherein the gaseous atmosphere did not contain HBr, such temperatures were in fact standard, or substantially so, for any given metal or combination of metals. For example, with the powdered iron, the temperature used was about 2000° F. This standard temperature, chosen in accordance with the prior art, may be defined as that at which at least one metal present is brought to the point of incipient fusion. At the same time, these standard temperatures were always less than the melting point of the highest melting metal present. As such, therefore, the temperatures varied substantially depending upon the composition of the metal or metals contained in the part being heat treated. For the purpose of the present discussion, these prior art sintering temperatures in an atmosphere in which HBr was absent may be termed standard temperatures. Such standard temperatures may be found in many textbooks and articles treating this subject matter.

In accordance with the present invention, the process may be practiced at the standard temperature as aforesaid for the material in question and thereby greatly enhanced physical characteristics obtained in the final article, particularly tensile strength, and elongation. This practice represents one embodiment of the present invention.

Another embodiment of the present invention from this point of view is the corresponding operation at substantially reduced temperatures in respect to standard temperatures as aforesaid respectively. At such reduced temperatures, which are substantially less than the standard temperatures for any given metal composition respectively, at least as great or as desirable physical properties may be attained in the final product as would result from the practice of prior art processes with respect to the same type article. For example, taking the case of an iron article, the standard temperature of the prior art is about 2000° F. when using an atmosphere containing no HBr. In accordance with the present invention, a final article formed from iron powder can be prepared using a sintering temperature of about 1600° F. and having at least as desirable physical properties of strength and elongation. Thus, in accordance with this embodiment of the process of the invention, substantially less heat is required, with a corresponding saving in the cost of the heat and in wear and tear on the equipment used incident to the use of higher temperatures.

Intermediate practices may also be used in accordance with the present invention using temperatures between the standard temperature and the lowest temperature possible as aforesaid, which may be expressed as somewhat lower than the standard temperatures, and attaining results somewhat more desirable than those attainable in accordance with the prior art practices.

It is also contemplated in accordance with the present invention, that a predetermined temperature may be used, when heat treating a metallic article including two or more metals, which predetermined temperature will be below the melting point of the highest melting point of one or more lower melting metals present. Using this

phase of the invention, some one or more of the lower melting metals may, in fact, be caused to fuse, thus serving to bind together the unfused particles of the higher melting metal.

In accompanying drawings there is illustrated graphically some of the desirable results of the present invention, so that these results may be visualized more easily than could be done from mere tabulated results.

In the drawings:

Figure 1 is a plot showing the relation between tensile strength and sintering temperature in iron articles previously pressed at 50,000 p. s. i. and with different concentrations of HBr present in the atmosphere during sintering, a legend below the plot indicating the percent HBr used for each curve; and

Fig. 2 is a plot showing the relationship between tensile strength and HBr concentration (by volume) in the gaseous atmosphere during sintering, the curves being shown for different temperatures as marked respectively thereon and the material used for all curves being iron powder pressed at 50,000 p. s. i.

In the accompanying drawings, a comparison is given with the prior art which is that condition represented by 0% HBr. It will be noted from the several curves that substantially enhanced results as to tensile strength are obtained when progressively greater concentrations of HBr are present in the gases from about 1% up to about 5%; and that these results are different from those obtainable by prior art practice to a substantial and surprising extent. While the data forming the bases for the curves shown in the drawings was obtained using powdered iron test pieces, similar results are obtainable using other metals or combinations thereof, as set forth hereinafter.

The data illustrated in Figs. 1 and 2 is set forth in tabular form in Table I below:

TABLE I

[Iron powder pressed at 50,000 p. s. i. before heat treatment]

| Percentage HBr in Atmosphere by Volume | Tensile Strength in p. s. i. | Temperature, °F. | Elongation in Percent |
|----------------------------------------|------------------------------|------------------|-----------------------|
| 0                                      | 10,240                       | 1,600            | 4.0                   |
| 0.5                                    | 8,640                        | 1,600            | 2.7                   |
| 1.0                                    | 12,050                       | 1,600            | 4.7                   |
| 5.0                                    | 16,500                       | 1,600            | 8.7                   |
| 10.0                                   | 15,610                       | 1,600            | 8.0                   |
| 15.0                                   | 15,610                       | 1,600            | 8.7                   |
| 0                                      | 10,340                       | 1,800            | 3.3                   |
| 0.5                                    | 8,580                        | 1,800            | 2.7                   |
| 1.0                                    | 13,400                       | 1,800            | 4.7                   |
| 5.0                                    | 17,680                       | 1,800            | 7.8                   |
| 10.0                                   | 18,080                       | 1,800            | 8.0                   |
| 15.0                                   | 17,450                       | 1,800            | 6.7                   |
| 0                                      | 13,900                       | 2,000            | 5.3                   |
| 0.5                                    | 11,570                       | 2,000            | 4.7                   |
| 1.0                                    | 15,670                       | 2,000            | 6.0                   |
| 5.0                                    | 19,270                       | 3,000            | 8.0                   |
| 10.0                                   | 19,250                       | 2,000            | 6.7                   |
| 15.0                                   | 19,720                       | 2,000            | 5.3                   |

From Table I above, it will be noted that the results obtained in terms of tensile strength and elongation for the tests made using 0.5% HBr by volume, are lower than the results obtained by sintering in pure hydrogen. On the other hand, in the preferred higher concentrations of at least about 5% HBr, positively improved results are obtained in respect to the prior art wherein no HBr was used.

The application of the process of the invention to various powdered metals including metals other than iron may be illustrated by the following examples:

#### Example 1

Powdered metal parts were tested consisting of 92.5% iron powder and 7.5% copper powder (by weight), produced by mixing copper and iron powders in these proportions and pressing the mixed powders to shape at

50,000 p. s. i. Some of these parts were then sintered in pure hydrogen at 1800° F. for one hour. Other parts produced in the same way, but containing 90% iron and 10% copper (by weight), were sintered for the same time and at the same temperature in an atmosphere consisting of 95% hydrogen and 5% HBr gas by volume. The tensile strength of the parts sintered in pure hydrogen was 16,000 p. s. i. and their elongation was 1.5%. The copper-iron parts that were sintered in the atmosphere containing 5% HBr as aforesaid had a tensile strength of 21,200 p. s. i. and elongation of 2.0%. Even though the composition of these two types of parts with respect to iron and copper differed slightly, this example illustrates that sintering in an atmosphere containing HBr has a beneficial effect on the tensile strength of mixed copper-iron powders. The differences in tensile strength was much greater than could be attained by the slight differences in composition.

#### Example 2

Metal parts were prepared by mixing 97% of iron powder and 3% of nickel powder (by weight) and pressing the mixed powders at 50,000 p. s. i. Some of these parts were sintered for one hour in an atmosphere of pure hydrogen at 1800° F., while others, having the same composition, were sintered under the same conditions of time and temperature in an atmosphere consisting of 95% hydrogen and 5% HBr gas by volume. The parts sintered in pure hydrogen had a tensile strength of 11,280 p. s. i. and an elongation of 3.1%, while the other parts of the same composition sintered in the atmosphere containing HBr aforesaid had a tensile strength of 12,800 p. s. i. and an elongation of 3.5%.

#### Example 3

Powdered metal parts (simulating bronze) consisting of 90% copper powder and 10% tin powder (by weight), were prepared by mixing these two powders and pressing the mixed powders to a desired shape at 50,000 p. s. i. Some of these parts were sintered for one hour at a temperature of 1475° F., while others were sintered under the same conditions in an atmosphere consisting of 95% hydrogen and 5% HBr gas by volume. These parts sintered in pure hydrogen had a tensile strength of 14,040 p. s. i. and an elongation of 0%, while those sintered in the atmosphere including HBr gas aforesaid had a tensile strength of 28,700 p. s. i. and an elongation of 17.0%. In this mixture particularly, the advantage of sintering in HBr-containing atmosphere are strikingly illustrated, especially with regard to improving the percent elongation.

#### Example 4

As an example of the application of the invention with gases of a non-reducing, neutral character, the results of sintering powdered iron parts in a nitrogen atmosphere are set forth below. Samples were prepared from the same type of powdered iron employed in the tests reported in Figs. 1 and 2 and in Table I above, by pressing the iron powder to a desired shape at 50,000 p. s. i. Some of the test pieces so prepared were sintered for one hour at 1800° F. in an atmosphere of pure nitrogen, while others were sintered under the same conditions in an atmosphere consisting of 90% nitrogen and 10% HBr gas by volume. The test pieces sintered in the atmosphere of pure nitrogen had a tensile strength of 11,130 p. s. i. and an elongation of 0.9%; while those sintered in an atmosphere containing HBr had a tensile strength of 16,600 p. s. i. and an elongation of 8.0%. Thus, it will be seen that as compared with using a neutral atmosphere such as nitrogen, the addition of HBr substantially enhanced the physical properties of a heat treated powdered metal part. However, it will be noted by comparison with the data set forth in Table I, that the increase in tensile strength is not as great as when the

heat treatment is carried out in an atmosphere containing hydrogen.

During the tests on the heat treatment of iron articles in an atmosphere of nitrogen and HBr, the presence of FeBr<sub>2</sub> was observed in the exit gases. It is believed that during the process, the beneficial effects of the HBr were partially counteracted by the formation and subsequent volatilization of FeBr<sub>2</sub>, which weakened the product physically to some extent. However, this undesired bromidization did not take place to such an extent as to prevent the HBr from enhancing the tensile strength of the part as compared with a similar part sintered in an atmosphere containing no HBr. This example is further submitted to illustrate the beneficial effects of the presence of a reducing gas such as hydrogen.

*Example 5*

This example illustrates the use of the present process in connection with a pre-alloyed brass powder consisting of 90% copper and 10% zinc by weight. Zinc is a metal which is relatively easy to bromidize as compared to such metals as iron, nickel, copper, etc. Test samples were prepared from the pressed alloy powder, described above, by pressing at 50,000 p. s. i. Some of these samples were sintered for one hour in an atmosphere of pure hydrogen at temperature of 1620° F., while others were sintered under the same conditions in an atmosphere consisting of 95% hydrogen and 5% HBr gas by volume. The parts sintered in the atmosphere of pure hydrogen had a tensile strength of 10,150 p. s. i. and an elongation of 3.6%; while those sintered in the HBr-containing atmosphere had a tensile strength of only 8,680 p. s. i. and an elongation of only 2.5%. The decrease in tensile strength and percentage elongation caused by the sintering in a HBr-containing atmosphere is believed to be due to the fact that the relatively reactive zinc-containing powder combines with the HBr gas to form zinc bromide, which volatilizes at the temperatures employed, leaving the structure of the part substantially weakened. This material is not to be considered as within the scope of the present invention.

*Example 6*

In order to investigate the effect of the presence of an admixed solid halide on the physical properties of heat treated powdered metal parts, several samples were prepared by mixing various amounts of solid anhydrous FeBr<sub>2</sub> with the powdered iron in forming the part being treated. It was contemplated that by sintering such a mixture in a hydrogen-containing atmosphere, the reaction between hydrogen and FeBr<sub>2</sub> would produce gaseous HBr, so that the present process might be carried out in this way with equivalent results. The actual results of such tests are set forth in Table II below.

TABLE II

Iron powder having different amounts of admixed FeBr<sub>2</sub> were pressed at 50,000 p. s. i. before heat treatment:

| Percent Solid FeBr <sub>2</sub> in Mixture | Temperature, ° F. | Tensile Strength, p. s. i. |
|--------------------------------------------|-------------------|----------------------------|
| 0.....                                     | 1,800             | 10,050                     |
| 0.5.....                                   | 1,800             | 7,160                      |
| 1.0.....                                   | 1,800             | 6,460                      |

From the data given in Table II, it will be seen that the effect of adding solid ferrous bromide is to decrease, rather than to increase, the tensile strength of the parts. The process of the present invention does not include sintering powdered metal parts in which solid halides are admixed with the powdered metal in lieu of otherwise supplying gaseous HBr in the atmosphere in which the parts are heat treated.

When one sample of Swedish iron powder, compacted

at 50,000 p. s. i. was sintered in an atmosphere of pure hydrogen, at 1800° F., the resulting article had a tensile strength of about 10,000 p. s. i. A second sample of the same Swedish iron powder having 0.5% FeBr<sub>2</sub> thoroughly admixed therewith was compacted at the same pressure of 50,000 p. s. i. and then sintered at the same temperature of 1800° F., resulting in a test piece having a tensile strength of only about 7000 p. s. i. A third sample of the same powder, having the same 0.5% admixed FeBr<sub>2</sub> and compacted at the same pressure of 50,000 p. s. i., was then sintered at the same temperature of 1800° F., this time in an atmosphere consisting of 95% hydrogen and 5% HBr (both by volume). This sample had a tensile strength, measured by the same test, of about 9800 p. s. i. This demonstrates that while the presence of admixed bromide has an undesired effect of lowering the tensile strength of the final article, the presence in the sintering atmosphere of HBr derived from a source other than reaction between admixed bromide and a reducing gas constituent of the sintering atmosphere, will result in enhancing the tensile strength as contrasted with the results obtainable when using a sintering atmosphere in which HBr is absent. It is reasonably to be concluded, therefore, that where the amount of admixed bromide in the metallic body being sintered is minimized and is not too great, the desirable effects of the presence of HBr in the sintering atmosphere may not only compensate for the undesired results due to admixed bromide, but may give superior results, notwithstanding a minor diminution of the tensile strength by small amounts, as traces, of admixed bromide.

While the process of the present invention has been disclosed as applied to a limited number of the many possible combinations to which it is applicable, the principles herein set forth are applicable generally within the limits stated. It is intended that the appended claims shall be construed to cover all reasonable equivalents as will occur to those skilled in the art from the foregoing particular disclosure, and that the claims be construed validly as broadly as the state of the prior art permits.

What is claimed is:

1. The process of making metallic parts with a metallic material of at least one of the relatively difficultly bromidizable powdered metals selected from the group which consists of iron, nickel, cobalt, copper, cadmium, lead, tin and molybdenum, and wherein the amount of bromides intermixed with said metallic material is minimized, said process comprising the step of heat treating said material in a non-oxidizing atmosphere, establishing and maintaining in said atmosphere a concentration of at least about 1% of gaseous HBr by volume, by supplying gaseous HBr to said atmosphere from a source independent of any intermixed bromine-containing material in said solid material, said heat treating being effected, by raising the temperature of said material to the point at which at least one metal present is brought to the point of incipient fusion in said atmosphere.

2. The process in accordance with claim 1, wherein the volume concentration of gaseous HBr in said atmosphere is from about 1% to about 15%.

3. The process in accordance with claim 1, wherein the volume concentration of gaseous HBr in said atmosphere is about 5% to about 15%.

4. The process in accordance with claim 1, wherein said non-oxidizing atmosphere contains hydrogen.

5. The process in accordance with claim 1, wherein said non-oxidizing atmosphere consists essentially of a mixture of gaseous HBr and hydrogen.

6. The process in accordance with claim 1, wherein said non-oxidizing atmosphere consists essentially of a mixture of gaseous HBr and nitrogen.

7. The process in accordance with claim 1, wherein said heat treating is carried on at substantially the same

temperature at which some one metal present in said metallic material will sinter in the same atmosphere without HBr present therein, so as to produce a part having enhanced physical properties in respect to the corresponding physical properties of such a part sintered in the same atmosphere but without HBr therein.

8. The process in accordance with claim 1, wherein said heat treating is carried on at a temperature substantially below that temperature at which some one metal present in said metallic material would sinter by being brought to the point of incipient fusion in the same atmosphere in the absence of HBr therein, so as to produce a part having substantially as desirable physical properties as the part would have if sintered by being brought to the point of incipient fusion in the same atmosphere in the absence of HBr therein at said temperature at which some metal present would sinter as aforesaid in the absence of HBr.

9. The process in accordance with claim 1, wherein said heat treating is carried on at a temperature somewhat lower than that at which some one metal present in said metallic material would sinter by being brought to the point of incipient fusion in the same atmosphere in the absence of HBr therein, so as to produce a part having somewhat enhanced physical properties in respect to the properties which would be present in a similar part sintered as aforesaid in the same atmosphere in the absence of HBr at said temperature at which this metallic material would sinter as aforesaid in such atmosphere in which HBr was absent.

10. The process in accordance with claim 1, wherein said metallic material is powdered iron, and wherein said atmosphere contains from about 5% to 15% gaseous HBr by volume.

11. The process in accordance with claim 1, wherein said metallic material is powdered iron.

12. The process in accordance with claim 1, wherein said metallic material consists of iron and nickel, and wherein said atmosphere contains about 5% gaseous HBr by volume, the temperature of the heat treatment being at least that at which nickel powder is brought to the point of incipient fusion.

13. The process in accordance with claim 1, wherein said metallic material consists of copper and tin, and wherein said atmosphere contains about 5% gaseous HBr by volume, the temperature of the heat treatment being at least that at which tin powder is brought to the point of incipient fusion.

14. The process in accordance with claim 1, wherein said metallic material consists of copper and iron, and wherein said atmosphere contains about 5% gaseous HBr by volume, the temperature of the heat treatment being at least that at which copper powder is brought to the point of incipient fusion.

15. The process of making metallic parts starting with a metallic material containing at least two of the rela-

tively difficultly bromidizable powdered metals selected from the group consisting of iron, nickel, cobalt, copper, cadmium, lead, tin and molybdenum, and wherein the amount of bromides intermixed with said metallic material is minimized, said process comprising the step of heat treating said material in a non-oxidizing atmosphere, establishing and maintaining in said atmosphere a concentration of at least about 1% of gaseous HBr by volume, by supplying gaseous HBr to said atmosphere from a source independent of any intermixed bromine-containing material in said solid material, said heat treating being effected by raising the temperature of said material to a point at least as high as that at which at least one metal present is brought to the point of incipient fusion in said atmosphere and below the temperature at which the highest melting metal present will melt.

16. The process of making metallic parts by powdered metallurgy practices, starting with a metallic material of at least one of the relatively difficultly bromidizable powdered metals selected from the group which consists of iron, nickel, cobalt, cadmium, lead, copper, tin and molybdenum, and wherein the amount of bromides intermixed with said metallic material is minimized, said process comprising the steps of compacting said metallic material at a predetermined pressure to a desired form for a part to be made, and heat treating said material in a non-oxidizing atmosphere, establishing and maintaining in said atmosphere a concentration of at least about 1% of gaseous HBr by volume, by supplying gaseous HBr to said atmosphere from a source independent of any intermixed bromine-containing material in said solid material, said heat treating being effected by raising the temperature of said material to a point at which at least one metal present is brought to the point of incipient fusion in said atmosphere.

17. As a new product, a metal article consisting essentially of sintered powdered metal selected from the group which consists of the metals: iron, nickel, cobalt, copper, cadmium, lead, tin, and molybdenum and mixtures and alloys consisting essentially of said metals, and wherein the amount of bromides intermixed with said metallic material is minimized, said article being prepared by the process of claim 1.

#### References Cited in the file of this patent

#### UNITED STATES PATENTS

|           |             |               |
|-----------|-------------|---------------|
| 2,199,418 | Redmond     | May 7, 1940   |
| 2,397,831 | Bellamy     | Apr. 2, 1947  |
| 2,431,690 | Hall et al. | Dec. 2, 1947  |
| 2,558,750 | Harrison    | July 3, 1951  |
| 2,593,943 | Wainer      | Apr. 22, 1952 |
| 2,585,819 | Moore       | Feb. 12, 1952 |

#### FOREIGN PATENTS

|         |               |                |
|---------|---------------|----------------|
| 592,404 | Great Britain | Sept. 17, 1947 |
|---------|---------------|----------------|